

# United States Patent Office

3,156,685

Patented Nov. 10, 1964

1

3,156,685

IMPROVED POLYMETHINE SENSITIZING DYES  
Jean Marie Nys and Henri Depoorter, Mortsel-Antwerp,  
Belgium, assignors to Gevaert Photo-Producten N.V.,  
Mortsel, Belgium, a Belgian company  
No Drawing. Filed July 3, 1961, Ser. No. 121,372  
Claims priority, application Great Britain June 20, 1957  
5 Claims. (Cl. 260—240.6)

This invention relates to new methine dyes and to their preparation and use as sensitizers for photographic silver halide emulsions, and to methods of sensitizing such emulsions by means of such sensitizing dyes.

A great number of methine dyes are known and many of them have been found to sensitize photographic emulsions in a variety of useful manners. These sensitizing methine dyes, however, when used in such emulsions leave in general a residual stain in the colloid image-bearing layers and/or in other photographic layers such as sub-layers or even in the film support of developed and fixed photographic elements. The staining effect is particularly troublesome in the case of photographic elements which are used in photo-mechanical processes, for example photographic negatives of the lithographic type which are to be corrected subsequently by a color mask image, and therefore a neutral tint is an absolute requirement. This staining effect is furthermore particularly objectionable in photographic papers since it is impossible, when such dye-sensitized emulsions are used, to obtain bright whites in a black-and-white picture or a true reproduction of the colors in a color picture. A light rose or yellow residual stain may further cause trouble when a finished photograph is exposed partly to full daylight, the other part being covered, so that under the influence of light the residual dye-stuff can bleach out, leaving an image which is partly white and partly colored.

It is therefore very important, when sensitizing photographic emulsions by dyes, to avoid this residual staining effect in finished photographic papers, in films of the lithographic type or in other finished photographs in which such stain is objectionable.

It is an object of the present invention to provide a new class of methine dyes which do not leave a residual stain in developed and fixed photographic elements. A further object is to provide methods for preparing these new dyes. Still another object is to provide silver halide emulsions sensitized with these new dyes. A still further object is to provide a practical and useful method for sensitizing silver halide emulsions which has the great advantage that, when such emulsions are coated on a suitable support, the exposed photographic element after development and fixing gives a finished photograph which is essentially free from any residual stain. Other objects will become apparent from a consideration of the description and examples.

It is common knowledge that the methine dyes are adsorbed on the silver halide crystals and on the particles of the colloid binder along the organic residue attached to the auxochrome nitrogen atom, that is the cyanine nitrogen atom which is linked through a conjugated carbon chain to another auxochrome group such as for example a nitrogen atom or a carbonyl, thiocarbonyl or cyano group.

It has now been found that sensitizing methine dyes, which are adsorbed on the silver halide crystals and on the hydrophilic water-permeable colloid binder along an organic residue bearing a hydrophilic group as defined more particularly hereinafter, do not leave an objectionable residual stain in the photographic layers after development and fixing of the exposed photographic element has been completed, independently of the water-solubility of the new methine dyes involved. It has been

2

found indeed that by introducing in the molecule of the methine dye an organic residue containing a hydrophilic group according to the invention, the residual stain is at all events completely avoided, although in many cases the water-solubility of the new dyes is not markedly changed and in some cases even diminished. In this way it was surprisingly discovered that some new methine cyanine dyes which contain an organic residue bearing a hydrophilic group according to the invention are considerably less water-soluble than the corresponding alkyl substituted dyes, but nevertheless left no residual stain in the finished photograph. The readiness with which the new methine dyes can be removed from the exposed photographic element during processing consequently has no direct relation with the solubility of the dyes involved but is or may be regarded as a result of a desorption phenomenon whereby in aqueous medium the dye molecules are withdrawn from the surface of the silver halide crystals and/or of the particles of the colloid binder on account of the great water-affinity of the organic residues containing the hydrophilic groups according to the invention. The existence of such desorption phenomena is known from adsorption chromatographic separation techniques where the solubility does not play a preponderant role either.

It is further known that methine dyes containing electro-negative groups in general are relatively poor sensitizers for photographic emulsions or even desensitizers for such emulsions and therefore not useful as practical photographic sensitizers.

It has now been found that the sensitizing power of the new methine dyes, which contain an organic residue bearing a hydrophilic group according to the invention, is not markedly reduced notwithstanding the high electro-negative value of the hydrophilic groups involved.

We have also found that the introduction into a methine dye of such an organic residue bearing a hydrophilic group as defined more particularly hereinafter clearly results in a shifting of the sensitization spectrum to the shorter wave-lengths and that these hypsochrome shifts can in some cases amount to 5-10  $\mu$ . In the case of orthochromatic emulsions this hypsochrome shifting may be very desirable to allow an extension of the spectrum composition of the light in the darkroom to physiologically clearer, that is shorter wave-lengths without the risk of fogging the emulsion; such an extension is inter alia required when treating photographic elements used for copying and/or photomechanical processes. If this shifting is undesirable, it can be remedied by adaption of the other elements constituting the methine dye, for example by changing a heterocyclic nucleus or by introducing a substituent into a nucleus or in the conjugated chain.

According to the present invention we provide new sensitizing methine dyes in which at least one heterocyclic nitrogen atom carries an organic residue of the following constitution:



wherein A and B each represents a hydrocarbon group.  
60 That residue linked to an auxochrome heterocyclic nitrogen atom of methine dye salts may have a betaine structure by intra-molecular ionization of the sulphonic acid group:



In the above formulae A preferably represents alkylene groups having from 1-4 carbon atoms such as methylene, ethylene, and propylene alone or coupled to a mono-nuclear arylene radical such as benzylene (phenylene methylene) and B preferably represents an alkylene group

having from 1-6 carbon atoms such as methylene, ethylene, propylene and butylene.

According to a further feature of the present invention we provide a photographic silver halide emulsion sensitized by incorporating therein at least one of the new methine dyes as hereinbefore defined. The present invention further includes a process for preparing high sensitive photographic silver halide emulsions which give, after development and fixing of the exposed photographic element, a finished photograph which is essentially free from any residual stain, which comprises treating a photographic silver halide emulsion with a sensitizing polymethine dye as defined herein and a light sensitive photographic element containing at least one silver halide emulsion layer sensitized according to the foregoing process.

The present invention also includes a method of preparing methine dyes, which method consists in treating a quaternary salt of a heterocyclic nitrogen base bearing at the nitrogen atom an organic residue of the following constitution:



wherein M represents an alkali metal atom, such as sodium, potassium or the like or an ammonium group and A and B have the same significance as set forth hereinbefore, by one of the methods known to be capable of converting the alkyl, aryl or aralkyl quaternary salt of such heterocyclic base into a methine dye. The word "known" is to be understood as designating methods in actual use or described in literature on the subject.

The quaternary salts employed in the present invention can be obtained by treating the corresponding heterocyclic nitrogen base with a compound of the general formula:



wherein X represents an acid residue such as for example a halogen atom such as Cl and Br, and M, A and B have the same significance as set forth hereinbefore. The heterocyclic nitrogen base and the compound of Formula I above are merely heated together to form the quaternary halide. Crude quaternary halides prepared in this manner may be converted, if desired, into other quaternary salts before employing them to prepare our new methine dyes.

The compounds of the general formula I wherein B represents a hydrocarbon radical containing a straight carbon chain of at least three carbon atoms may be prepared by heating together a compound of the general formula:



with a compound of the general formula:



wherein B<sub>1</sub> represents a hydrocarbon radical containing a straight chain of at least three carbon atoms and not more than 6 carbon atoms and containing preferably 3 or 4 carbon atoms and M, X and A have the same significance as set forth hereinbefore.

The compounds of the general formula I above wherein B represents a methylene radical may be prepared by heating together a compound of the general formula:



with a compound of the general formula:



wherein B<sub>2</sub> represents a methylene radical and X, A and M have the same significance as set forth hereinbefore.

The present application is a continuation-in-part of 75

our application Serial No. 742,713 filed June 18, 1958, now abandoned.

The following examples will serve to illustrate the method for preparing the intermediate compounds of the general Formula I above.

#### PREPARATION I

##### 3-Bromo-Acetoxy-Propane-1-Sulphonic Acid Sodium Salt



Sodium bromo-acetate (50 g.) and 3-hydroxypropane-1-sulphonic acid sultone (50 g.) are heated for six hours at 150° C. upon an oil-bath and with occasional stirring. After cooling, the mixture is washed with ether. Melting point 188° C.

#### PREPARATION II

##### 4-Bromo-Acetoxy-Butane-1-Sulphonic Acid Sodium Salt



Sodium bromo-acetate (100 g.) and 4-hydroxy-butane-1-sulphonic acid sultone (100 g.) are heated for six hours at 150° C. upon an oil-bath and with occasional stirring. After cooling the mixture is ground in a mortar and thoroughly washed with ether. Melting point 200° C.

#### PREPARATION III

##### Bromo-Acetoxy-Methane Sulphonic Acid Sodium Salt



Bromo-acetanhydride (21 g.) and sodium-hydroxymethane sulphonate (5.36 g.) are gently heated over a flame until at about 60° C. the reaction sets in. At this moment, the flame is removed and the temperature increases to about 110° C. When the reaction diminishes in intensity the mass is heated for some minutes at 120° C. After cooling, the reaction product is washed out with ether and purified by recrystallization from diluted ethanol or propanol. Melting point 243° C. (with decomposition).

The quaternary salts employed in the present invention can also be obtained by treating the corresponding quaternary salt, bearing at the nitrogen atom an organic residue of the following constitution:



wherein A has the same significance as set forth hereinbefore, and which may be prepared by treating the corresponding heterocyclic base with a compound of the general formula:



wherein X and A have the same significance as set forth hereinbefore, with a compound of the general formula:



wherein B<sub>1</sub> represents a hydrocarbon radical containing a straight carbon chain of at least three carbon atoms.

As suitable heterocyclic nitrogen bases, known to be convertible into a methine dyestuff, may be mentioned the heterocyclic nitrogen bases containing in the alpha or gamma-position to the nitrogen atom of the heterocyclic ring an alkyl, thioalkyl, beta-alkylthiovinyl, betahalogenovinyl, beta (N-methylanilino)-vinyl or beta-acyl-anilidovinyl group, which vinyl groups may carry a substituent, such as a lower alkyl group.

While the process of preparing the quaternary halides is subject to variation particularly in respect of the nature of the heterocyclic nitrogen bases, the nature of the compounds of the general Formula I above, the proportions of the reactants, the temperature, the time of reaction and the methods of isolation and purification of the quaternary halides, the following examples will serve to illustrate the method for preparing the quaternary halides.

## PREPARATION IV

2-Methyl-3-(Sodium Sulpho-Carbomethoxy-Methyl-Benzothiazolium Bromide



Bromo-acetoxymethane sulphonic acid sodium salt (3 g.) and 2-methyl benzothiazole (10 g.) are heated for eight hours at 105° C. and at times the mass is thoroughly stirred. After cooling the mixture is washed with ether. The product is very hygroscopic.

## PREPARATION V

2-Methyl-3-(Omega Sodium Sulpho-Carbopropoxy-Methyl)-Benzothiazolium Bromide



3-bromo-acetoxymethane sulphonic acid sodium salt (28.3 g.) and 2-methyl benzothiazole (20 g.) are heated for sixteen hours at 100° C. After cooling, the product is washed with ether. Melting point: 172° C.

## PREPARATION VI

2-Methyl-3-(Omega-Sodium Sulpho-Carbobutoxy-Methyl)-Benzothiazolium Bromide



A mixture of 4-bromo-acetoxymethane-1-sulphonic acid sodium salt (75 g.) and 2-methyl-benzothiazole (65 g.) is heated for 22 hours at 100° C. The mixture is thoroughly stirred from time to time and after cooling the resulting product is washed with ether. Melting point: 190° C.

## PREPARATION VII

2-Methyl-3-(Omega-Sodium Sulpho-Carbobutoxy-Methyl)-Benzoselenazolium Bromide



A mixture of 2-methylbenzoselenazole (30 g.) and 4-bromo-acetoxymethane-1-sulphonic acid sodium salt (30 g.), is heated for 18 hours at 100° C. After cooling, the reaction mixture is ground in a mortar and washed with ether. Melting point: 168° C.

## PREPARATION VIII

2-Methyl-3-(Omega-Sodium Sulpho-Carbopropoxy-Methyl)-Benzoselenazolium Bromide



3-bromo-acetoxymethane sulphonic acid sodium salt (28.3 g.) and 2-methyl-benzoselenazole (25 g.) are heated for twenty hours at 110° C. upon an oil-bath and after cooling washed with ether. Melting point: 170° C.

## PREPARATION IX

2-Methyl-3-(Omega-Sodium-Sulpho-Carbobutoxy-Methyl)-Thiazolinium Bromide



10 2-methyl-thiazoline (20.2 g.) and 4-bromo-acetoxymethane-1-sulphonic acid sodium salt (29.7 g.) are heated for six hours at 100° C. and after cooling the reaction product is ground and washed with ether. Melting point: 162° C.

## PREPARATION X

2-Methyl-4-(Omega-Sodium-Sulpho-Carbopropoxy-Methyl)-Thiazolinium Bromide



25 2-methyl-thiazoline (20.2 g.) and 3-bromo-acetoxymethane-1-sulphonic acid sodium salt (28.3 g.) are heated for five hours upon a boiling water bath, and, after cooling, the reaction product is washed with ether and further purified by dissolving in ethanol, treating with animal charcoal and precipitating with ether. Melting point: 30 170° C.

## PREPARATION XI

2-Methyl-3-(Omega-Sodium-Sulpho-Carbopropoxy-Methyl)-6-Methoxy-Benzothiazolium Bromide



35 A mixture of 2-methyl-6-methoxy-benzothiazole (24 g.) and 3-bromo-acetoxymethane-1-sulphonic acid sodium salt (28.3 g.) is heated for sixteen hours at 100° C. After cooling the reaction product is washed with ether. Melting point: 45 180° C.

## PREPARATION XII

2-Methyl-3-(Omega-Sodium Sulpho-Carbobutoxy-Methyl)-6-Methoxy-Benzothiazolium Bromide



50 55 2-methyl-6-methoxy-benzothiazole (18 g.) and 4-bromo-acetoxymethane-1-sulphonic acid sodium salt (23.7 g.) are heated for sixteen hours at 100° C. After cooling the reaction product is ground and washed with ether. Melting point: 60 160° C.

## PREPARATION XIII

2-Methyl-3-(Omega-Sodium Sulpho-Carbopropoxy-Methyl)-6-Methyl Benzothiazolium Bromide



65 70 75 A mixture of 2,6-dimethyl-benzothiazole (22 g.) and 3-bromo-acetoxymethane-1-sulphonic acid sodium salt (28.3 g.) is heated for sixteen hours at 100° C. After cooling, the resulting product is thoroughly washed with ether. Melting point: 172° C.

## PREPARATION XIV

2-Methyl-3-(Omega-Sodium Sulpho-Carbobutoxy-Methyl)-6-Methyl-Benzothiazolium Bromide



A mixture of 2,6-dimethyl-benzothiazole (20 g.) and 4-bromo-acetoxy-butane-1-sulphonic acid sodium salt (29.7 g.) is heated for sixteen hours at 100° C. After cooling the product obtained is washed with ether. Melting point: 174° C.

## PREPARATION XV

2-Methyl-3-(Omega-Sodium Sulpho-Carbobutoxy-Methyl)-5,6-Dimethyl-Benzothiazolium Bromide



2,5,6-trimethyl-benzothiazole (17.5 g.) and 4-bromo-acetoxybutane-1-sulphonic acid sodium salt (21.5 g.) are heated together for sixteen hours at 100° C. After cooling, the quaternary salt obtained is ground and washed with ether. Melting point: 180° C.

## PREPARATION XVI

2-Methyl-3-(Omega-Sodium Sulpho-Carbobutoxy-Methyl)-Benzoxazolium Bromide



2-methyl-benzoxazole (25 g.) and 4-bromo-acetoxybutane-1-sulphonic acid sodium salt (29 g.) are heated for sixteen hours at 130° C. After cooling the viscous reaction product solidifies by washing with ether. The product is very hygroscopic.

## PREPARATION XVII

2-Methyl-3-(Omega-Sodium Sulpho-Carbobutoxy-Methyl)-5-Phenyl-Benzoxazolium Bromide



2-methyl-5-phenyl-benzoxazole (25 g.) and 4-bromo-acetoxybutane-1-sulphonic acid sodium salt (29.7 g.) are heated for sixteen hours at 130° C. After cooling and washing with ether the sticky mass solidifies. The product is very hygroscopic.

## PREPARATION XVIII

2-Methyl-3-(Omega-Sodium Sulpho-Carbobutoxy-Methyl)-6-Methoxy-Benzoxazolium Bromide



2-methyl-6-methoxy-benzoxazole (20 g.) and 4-bromo-acetoxybutane-1-sulphonic acid sodium salt (29 g.) are heated for sixteen hours at 100° C. After cooling the reaction product is washed with ether. The product is very hygroscopic.

## PREPARATION XIX

2-Methyl-3-[p-(Omega-Sodium Sulpho-Carbobutoxy)-Benzyl]-Benzothiazolium Bromide



2-methyl-3-p-carboxybenzyl benzothiazolium bromide (5.3 g.) are brought into methanol (50 cm.³). After adding to this suspension a solution of sodium (0.23 g.) in methanol (10 cm.³), a violet solution is obtained, to which are added 8 g. butanesultone, dissolved in methanol (10 cm.³). The methanol is distilled off and the residue heated for two hours at 150-155° C. upon an oil-bath. After cooling, ether is added and the precipitate is ground. The product obtained is further purified by extracting with chloroform for five hours in a Soxhlet apparatus, and dried in a dessicator. The product is very hygroscopic.

## PREPARATION XX

2,5-Dimethyl-3-(Sodium Sulpho-Carbomethoxy-Methyl)-Benzothiazolium Bromide



A mixture consisting of 2,5-dimethyl-benzothiazole (4.5 g.) and sodium sulpho-carbomethoxy-methyl bromide (6 g.) is heated for 24 hours at 110° C. in a drying oven. The product is washed with ether, ground, sucked off and dried in vacuum.

## PREPARATION XXI

2,6-Dimethyl-3-(Sodium-Sulpho-Carbomethoxy-Methyl)-Benzothiazolium Bromide



A mixture consisting of 2,6-dimethylbenzothiazole (4.5 g.) and sodium sulpho-carbomethoxymethyl bromide (6 g.) is heated for 24 hours at 110° C. in a drying oven. The product obtained is washed with ether, ground and sucked off. Melting point: 178° C.

## PREPARATION XXII

1-Ethyl-2-Methyl-3-(Sodium Sulpho-Carbomethoxy-Methyl)-5,6-Dichloro-Benzimidazolium Bromide



1-ethyl-2-methyl-5,6-dichlorobenzimidazole (7 g.) and bromo-acetoxymethane sulphonic acid sodium salt 4.45 g.) are heated for 24 hours at 110° C., chilled and washed twice with acetone (10 cm.³) and once with ether (10 cm.³).

## PREPARATION XXIII

2,4-Dimethyl-3-(Sodium Sulpho-Carbomethoxy-Methyl)-Thiazolium Bromide



2,4-dimethylthiazole (8 g.) and bromo-acetoxymethane sulphonic acid sodium salt (7.65 g.) are heated for 18 hours at 110° C., chilled and washed with ether.

As stated hereinbefore, the new methine dyestuffs according to the present invention may be obtained starting from the new heterocyclic quaternary salts by application of the usual condensation methods known to those skilled in the art.

The following description of some methods for preparing the new methine dyes is not complete and therefore is not to be regarded as limiting the scope of our invention but merely as a survey of the most usual condensation methods.

The new asymmetric cyanine dyes according to the present invention can be prepared by condensing a cyclammonium quaternary salt of the following general formula:



wherein Z represents the non-metallic atoms to complete a heterocyclic nucleus containing 5 to 6 atoms in the heterocyclic ring of the type known in cyanine dyes, such as those selected from the group consisting of those of the thiazole series (e.g. thiazole, 4-methylthiazole, 4-phenylthiazole, 5-methylthiazole, 5-phenylthiazole, 4,5-dimethylthiazole, 4,5-diphenylthiazole, 4-(2-thienyl)-thiazole, etc.), those of the benzothiazole series (e.g. benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromo-benzothiazole, 6-bromobenzothiazole, 4-phenyl-benzothiazole, 5-phenylbenzothiazole, 4-methoxybenzothiazole, 5-methoxybenzothiazole, 6-methoxybenzothiazole, 5-iodo-benzothiazole, 6-iodobenzothiazole, 4-ethoxybenzothiazole, 5-ethoxybenzothiazole, 4,5,6,7-tetrahydrobenzothiazole, 5,6-dimethoxybenzothiazole, 5,6-dioxymethylenebenzothiazole, 5-hydroxybenzothiazole, 6-hydroxybenzothiazole, 5,6-dimethylbenzothiazole), those of the naphthothiazole series (e.g. naphtho[2,1-d]thiazole, naphtho[1,2-d]thiazole, 5-methoxynaphtho[1,2-d]thiazole, 5-ethoxy-naphtho[1,2-d]thiazole, 8-methoxynaphtho[2,1-d]thiazole, 7-methoxynaphtho[2,1-d]thiazole), those of the thiophenothieno[7',6'-d]thiazole series (e.g. 4'-methoxythiophenothieno[7',6'-d]thiazole), those of the oxazole series (e.g. 4-methyloxazole, 5-methyloxazole, 4-phenyloxazole, 4,5-diphenyloxazole, 4-ethyloxazole, 4,5-dimethyloxazole, 5-phenyloxazole), those of the benzoxazole series (e.g. benzoxazole, 5-chlorobenzoxazole, 5-methylbenzoxazole, 5-phenylbenzoxazole, 6-methylbenzoxazole, 5,6-dimethylbenzoxazole, 4,6-dimethylbenzoxazole, 5-methoxybenzoxazole, 6-methoxybenzoxazole, 5-hydroxybenzoxazole, 6-hydroxybenzoxazole), those of the naphthoxazole series (e.g. naphtho[2,1-d]oxazole, naphtho[1,2-d]oxazole), those of the selenazole series (e.g. 4-methylselenazole, 4-phenylselenazole), those of the benzoselenazole series (e.g. benzoselenazole, 5-chlorobenzoselenazole, 5-methoxybenzoselenazole, 5-hydroxybenzoselenazole, 4,5,6,7-tetrahydrobenzoselenazole), those of the naphthoselenazole series (e.g. naphtho 2,1-d selenazole, naphtho 1,2-d selenazole), those of the thiazoline series (e.g. thiazoline, 4-methylthiazoline, 4-hydroxymethyl-4-methylthiazoline, 4,4-bis-hydroxymethylthiazoline, 4-acetoxymethyl-4-methylthiazoline, 4,4-bis-acetoxymethylthiazoline), those of the thiazolidine series (e.g. 2-benzothiazolylidene-4-thiazolidone), those of the oxazoline series (e.g. oxazoline, 4-hydroxymethyl-4-methyloxazoline, 4,4-bis-hydroxymethyl-oxazoline, 4-acetoxymethyl-4-methyloxazoline, 4,4-bis-acetoxymethyloxazoline), those of the oxazolidine series, those of the selenazoline series (e.g. selenazoline), those of the 2-quinoline series (e.g. the quinoline, 3-methylquinoline, 5-methylquinoline, 7-methylquinoline, 8-methylquinoline, 6-chloroquinoline, 8-chloroquinoline, 6-methoxyquinoline, 6-ethoxyquinoline, 6-hydroxyquinoline, 8-

hydroxyquinoline etc.), those of the 4-quinoline series (e.g. quinoline, 6-methoxyquinoline, 7-methylquinoline, 8-methylquinoline), those of the 1-isoquinoline series (e.g. isoquinoline, 3,4-dihydroisoquinoline), those of the 3-isquinoline series (e.g. isoquinoline), those of the 3,3-dialkylindolenine series (e.g. 3,3-dimethylindolenine, 3,3,5-trimethylindolenine, 3,3,7-trimethylindolenine), those of the pyridine series (e.g. pyridine, 5-methylpyridine), those of the benzimidazole series (e.g. 1-ethylbenzimidazole, 1-phenylbenzimidazole, 1-ethyl-5,6-dichlorobenzimidazole, 1-hydroxyethyl-5,6-dichlorobenzimidazole, 1-ethyl-5-chlorobenzimidazole, 1-ethyl-5,6-dibromobenzimidazole, 1-ethyl-5-chloro-6-aminobenzimidazole, 1-ethyl-5-chloro-6-bromobenzimidazole, 1-ethyl-5-phenylbenzimidazole, 1-ethyl-5-fluorobenzimidazole, 1-ethyl-5-cyanobenzimidazole, 1-ethyl-5-chloro-6-cyano benzimidazole, 1-ethyl-5-fluoro-6-cyano benzimidazole, 1-ethyl-5-acetyl-benzimidazole, 1-ethyl-5-chloro-6-fluorobenzimidazole, 1-ethyl-5-carboxybenzimidazole, 1-ethyl-7-carboxybenzimidazole, 1-ethyl-5-carbethoxybenzimidazole, 1-ethyl-5-sulphonamidobenzimidazole, 1-ethyl-5-N-ethylsulphonamidobenzimidazole; X represents an acid radical of the type used in the cyanine dyes, such as chloride, bromide, iodide, perchlorate, benzenesulphonate, potassiumulphonate, methylsulphate, ethylsulphate etc.;

n represents 1 or 2 and

M, B and A have the same significance as set forth hereinbefore,

with a cyclammonium quaternary salt represented by the following Formula III:



wherein:

R<sub>1</sub> represents an alkyl group of the formula C<sub>r</sub>H<sub>2r+1</sub> wherein r represents a positive integer from 1 to 4 such as methyl, ethyl, propyl, isopropyl, butyl, isobutyl, an unsaturated aliphatic radical such as allyl, a hydroxy substituted alkyl radical such as β-hydroxyethyl, an aralkyl radical such as benzyl, a substituted aralkyl radical such as carboxy benzyl, a mononuclear aryl group such as phenyl, a substituted mononuclear aryl group such as carboxyphenyl, or a radical of the formula



as described above.

Z<sub>1</sub> represents the non-metallic atoms to complete a heterocyclic nucleus containing 5 to 6 atoms in the heterocyclic ring such as those described for Z,

n<sub>1</sub> represents 1 or 2,

X<sub>1</sub> represents an acid residue as known in cyanine dyes and

D represents an alkylmercapto, an arylmercapto, a beta-arylaminovinyl, a delta-arylmino-1,3-butadienyl, a beta-alkylmercaptovinyl, a beta-arylmercaptovinyl or a beta-acetanilidovinyl group, which vinyl groups may carry a substituent, such as methyl, benzyl or phenyl.

The condensations are advantageously carried out in the presence of a basic condensing agent, for example a trialkylamine such as triethylamine, a dialkylaniline, a heterocyclic tertiary amine such as pyridine, N-alkylpiperidine or the like.

The new symmetrical cyanine dyes according to the present invention can be prepared by condensing a cyclammonium quaternary salt represented by the general Formula II above with an ortho carboxylic acid alkyl ester, such as ethyl ortho-formate and ethyl ortho-acetate, advantageously in the presence of a carboxylic acid anhydride, for example acetic anhydride.

The new cyclammonium quaternary salts represented

## 11

by the general Formula II above can further be condensed with a compound represented by the following formula:



wherein

*t* represents an integer from 1 to 3,

Ar represents an aryl group and

$\text{L}_1$  and  $\text{L}_2$  each represents a methine group.

The aryl-amino-vinyl intermediates, or vinylene homologues thereof thus obtained can be transformed into the corresponding acetarylido derivatives by boiling with acetic anhydride, which can be condensed to unsymmetrical cyanine dyes with cyclammonium quaternary salts containing a methyl group in alpha or gamma position to the nitrogen atom. The condensations are advantageously carried out in the presence of a basic condensing agent as set forth above.

The most valuable methine dyes of the present invention may be represented by one of the two general Formulae A and B:

A.



B.



wherein:

$\text{Z}''$  and  $\text{Z}'$  each represents the non-metallic atom necessary to complete a heterocyclic nitrogen nucleus of the type contained in cyanine dyes,

$n'$  and  $n''$  each represents a positive integer from 1 to 2,

$d$  represents a positive integer from 1 to 3,

R represents a member selected from the group consisting of a hydrogen atom, and lower alkyl radical,

X represents an acid radical of the type used in cyanine dyes,

R'' represents a radical of the type contained in cyanine dyes as substituent on the cyanine nitrogen atom,

R' represents a radical of the formula



and

R''' represents a radical of the formula



in said radicals, R' and R'''  $p$  representing a positive integer from 1 to 6, M representing an alkali metal atom or cation such as ammonium and A representing a member selected from the group consisting of a lower alkylene radical or an arylene alkylene radical such as a benzylene radical.

The following examples will serve to illustrate further the manner of obtaining our new methine dyes.

## EXAMPLE 1

The dyestuff anhydro-[2-(ethyl-benzothiazole)]-[2-[3-(sulpho-carbomethoxy-methyl)-benzothiazole]]-mesomethyl-trimethinecyanine hydroxide, having the formula:



is prepared as follows:

2-methyl-3-(sodium sulpho-carbomethoxy-methyl)-benzothiazolium bromide (2 g.) and 2-( $\beta$ -methyl- $\beta$ -methyl-

10  
5

mercapto-vinyl)-3-ethyl benzothiazolium methylsulphate (1.8 g.) are dissolved in 200 cm.<sup>3</sup> ethanol and after adding 1.4 cm.<sup>3</sup> triethylamine boiled for twenty minutes. After cooling, the dyestuff is precipitated with ether and purified by recrystallization from propanol. Absorption maximum: 550 m $\mu$ .

A silver bromo-iodide emulsion containing per kg. 20 mg. of this dyestuff is sensitized to 650 m $\mu$  with a broad maximum at 590 m $\mu$ .

## EXAMPLE 2

The dyestuff anhydro-[2-(3-ethyl-selenazoline)]-[2-[3-(omega - sulpho - carbopropoxy - methyl) - benzothiazole]]-trimethinecyanine hydroxide, having the formula:



is prepared as follows:

2-methyl-3-(omega-sodium sulpho-carbopropoxy-methyl)-benzothiazolium bromide (8.65 g.) and 2-( $\beta$ -acetanilido-vinyl)-3-ethylselenazolium iodide (9 g.) are dissolved in 100 cm.<sup>3</sup> methanol. After cooling the solution at 0° C., 5.6 cm.<sup>3</sup> triethylamine are added drop by drop and after one hour stirring under ice cooling the dyestuff is sucked off and recrystallized three times from ethanol. Absorption maximum: 506 m $\mu$ .

A silver chloride emulsion containing per kg. 20 mg. of this dyestuff is sensitized to 580 m $\mu$  with a broad maximum at 540-545 m $\mu$ .

## EXAMPLE 3

The dyestuff anhydro-[2-(3-ethyl-benzoselenazole)]-[2-[3-(omega - sulpho - carbopropoxy - methyl)-benzo-selenenazole]]-mesomethyl-trimethinecyanine hydroxide, having the formula:



is prepared as follows:

2-methyl-3-(omega-sodium sulpho-carbopropoxy-methyl)-benzo selenazolium bromide (4.8 g.) and 2-( $\beta$ -methyl- $\beta$ -methylmercapto-vinyl)-3-ethyl-benzoselenazolium methylsulphate (4.1 g.) are dissolved in a mixture of 20 cm.<sup>3</sup> methanol and 20 cm.<sup>3</sup> pyridine. After adding drop by drop 1.4 cm.<sup>3</sup> triethylamine, the solution is brought to boiling temperature for five minutes. The dyestuff is precipitated with ether and purified by recrystallization from ethanol and methanol. Absorption maximum: 563 m $\mu$ .

A silver bromo-iodide emulsion containing per kg. 15 mg. of this dyestuff is sensitized to 655 m $\mu$  with a broad maximum at 600 m $\mu$ .

## EXAMPLE 4

The dyestuff anhydro-[2-(3-ethyl-thiazoline)]-[2-[3-(omega - sulpho - carbobutoxy - methyl)-benzothiazole]]-trimethinecyanine hydroxide, having the formula:



is prepared as follows:

2-methyl-3-(omega-sodium sulpho-carbobutoxy-methyl)-benzothiazolium bromide (4.60 g.) and 2-( $\beta$ -acetanilido-vinyl)-3-ethylthiazolium bromide (3.55 g.) are dissolved in warm ethanol (50 cm.<sup>3</sup>) and after cooling the solution

60

65

70

at 0° C., 1.4 cm.<sup>3</sup> trimethylamine are added. After stirring one hour under ice cooling, the dyestuff is sucked off and recrystallized from ethanol. Absorption maximum: 504 m $\mu$ .

A silver chloride emulsion containing per kg. 20 mg. of this dyestuff is sensitized to 580 m $\mu$  with a maximum at 530 m $\mu$ .

## EXAMPLE 5

The dyestuff anhydro-[2-(3-methyl-naphtho-1':2':4:5-thiazole)]-{2-[3-(omega-sulpho-carbobutoxy-methyl)-benzothiazole]}-monomethinecyanine hydroxide, having the formula:



is prepared as follows:

2-methyl-3-(omega-sodium-sulpho-carbobutoxy-methyl)-benzothiazolium bromide (4.5 g.) and 2-methylmercapto-3-methyl-naphtho-1':2':4:5-thiazolium methyl sulphate (3.6 g.) are dissolved in methanol (30 cm.<sup>3</sup>) and after cooling at 0° C., 2.8 cm.<sup>3</sup> triethylamine are added. After stirring for three hours at this temperature, the dyestuff is sucked off and recrystallized from diluted ethanol. Absorption maximum: 442 m $\mu$ .

A silver chloride emulsion containing per kg. 20 mg. of this dyestuff is strongly sensitized to 500 m $\mu$  with a sharp maximum at 470 m $\mu$ .

## EXAMPLE 6

The dyestuff anhydro-[2-(3-ethyl-benzothiazole)]-{2-[3-(omega-sulpho-carbobutoxy-methyl)-5-benzoxazole]}-trimethinecyanine hydroxide, having the formula:



is prepared as follows:

2-ethyl-3-(omega-sodium-sulpho-carbobutoxy-methyl)-5-phenyl benzoxazolium bromide (5.06 g.) and 2-( $\beta$ -acetanilidovinyl)-3-ethyl-benzothiazolium iodide (4.50 g.) are dissolved in 50 cm.<sup>3</sup> ethanol and after cooling the solution at 0° C., 1.4 cm.<sup>3</sup> triethylamine are added whilst stirring. After one hour the dyestuff is precipitated with ether and recrystallized three times from ethanol. Absorption maximum: 526 m $\mu$ .

A silver bromide emulsion containing per kg. 30 mg. of this dyestuff is strongly sensitized to 600 m $\mu$  with a high maximum at 550 m $\mu$ .

## EXAMPLE 7

The dyestuff anhydro-[2-(3-ethyl-benzoxazole)]-{2-[3-(omega-sulpho-carbobutoxy-methyl)-6-methoxy-benzothiazole]}-trimethinecyanine hydroxide, having the formula:



is prepared as follows:

2-methyl-3-(omega-sodium-sulpho-carbobutoxy-methyl)-6-methoxy benzothiazolium bromide (4.76 g.) and 2-( $\beta$ -acetanilidovinyl)-3-ethyl benzoxazolium iodide (4.34 g.) are dissolved in ethanol (50 cm.<sup>3</sup>) and after cooling the solution at 0° C., 1.4 cm.<sup>3</sup> triethylamine are added drop by drop whilst stirring. After standing for two

70

hours the dyestuff is completely precipitated with ether and recrystallized three times from ethanol. Absorption maximum: 530 m $\mu$ .

A silver bromide emulsion containing per kg. 30 mg. of this dyestuff is sensitized to 600 m $\mu$  with a maximum at 500 m $\mu$ .

## EXAMPLE 8

The dyestuff anhydro-bis{2-[3-(omega-sulpho-carbobutoxymethyl)-benzoxazole]}-trimethinecyanine hydroxide, having the formula:



is prepared as follows:

2-methyl-3-(omega-sodium-sulpho-carbobutoxy-methyl)-benzoxazolium bromide (4.3 g.), ortho-ethyl formate (2.96 g.) and acetic anhydride (25 cm.<sup>3</sup>) are heated for ten minutes at boiling temperature. After cooling, the dyestuff crystallizes and is purified by recrystallizing three times from ethanol. Absorption maximum: 485 m $\mu$ .

A silver chloride emulsion containing per kg. 30 mg. of this dyestuff is strongly sensitized to 560 m $\mu$  with a high maximum at 525 m $\mu$ .

## EXAMPLE 9

The dyestuff anhydro-bis{2-[3-(omega-sulpho-carbobutoxymethyl)-5,6-dimethylbenzothiazole]}-trimethinecyanine hydroxide, having the formula:



is prepared as follows:

2-methyl-3-(omega-sodium-sulpho-carbobutoxy-methyl)-5,6-dimethylbenzothiazolium bromide (4.74 g.) or orthoethyl formate (2.96 g.) and acetic anhydride (25 cm.<sup>3</sup>) are heated for fifteen minutes at boiling temperature. After cooling, the dyestuff crystallizes and is purified by recrystallizing three times from methanol. Absorption maximum: 570 m $\mu$ .

A silver bromo iodide emulsion containing per kg. 25 mg. of this dyestuff is sensitized to 670 m $\mu$  with a maximum at 590 m $\mu$ .

## EXAMPLE 10

The dyestuff anhydro-[3-n-propyl-thiazoline]-{2-[3-(sulpho-carbomethoxy-methyl)-benzothiazole]}-trimethinecyanine hydroxide, having the formula:



is prepared as follows:

2-methyl-3-(sodium-sulpho-carbomethoxy-methyl)-benzothiazolium bromide (4 g.) is dissolved in methanol (25 cm.<sup>3</sup>). After addition of 2-( $\beta$ -acetanilidovinyl)-3-n-propyl-thiazolium iodide (4.9 g.) and triethylamine (2.8 cm.<sup>3</sup>), the solution is cooled at 0° C. for ninety minutes. The dyestuff is sucked off and recrystallized from a mixture ethanol-water. Absorption maximum: 504 m $\mu$ .

A silver chloride emulsion containing per kg. 20 mg. of this dyestuff is sensitized to 575 m $\mu$  with a maximum at 530 m $\mu$ .

## EXAMPLE 11

The dyestuff anhydro-[2-(3-ethylthiazoline)]-{2-[3-

(sulpho - carbomethoxy-methyl) - 5 - methyl-benzothiazole]-trimethinecyanine hydroxide, having the formula:



is prepared as follows:

2,5-dimethyl-3-(sodium sulpho-carbomethoxymethyl)-

5

sucked off and crystallized from ethanol. Absorption maximum: 506 m $\mu$ .

A silver chloride emulsion containing per kg. 20 mg. of this dyestuff is sensitized to 600 m $\mu$  with a maximum at 540 m $\mu$ .

## EXAMPLE 14

The dyestuff anhydro{2 - [3 - sulpho - carbomethoxy - [5 - (3 - ethylrhodanine) - 2] - {2 - [3 - p-(omega-sulpho-carbobutoxy) - benzyl - benzothiazole]} alpha' - benzyl - dimethine rhodacyanine hydroxide, having the formula:



benzothiazolium bromide (4.2 g.) and 2-( $\beta$ -acetanilidovinyl)-3-ethyl thiazolinium bromide (3.5 g.) are dissolved in methanol (25 cm $^3$ ) and the solution is cooled at 0° C. 2.8 cm $^3$  triethylamine are added drop by drop and after one hour stirring under ice-cooling the dyestuff is sucked off and recrystallized three times from a mixture ethanol-water. Absorption maximum: 508 m $\mu$ .

A silver chloride emulsion containing per kg. 15 mg. of this dyestuff is sensitized to 590 m $\mu$  with a broad maximum at 540 m $\mu$ .

## EXAMPLE 12

The dyestuff anhydro-[2-(3-ethylthiazoline)]-{2 - [3 - (sulpho-carbomethoxy - methyl) - 6 - methylbenzothiazole]}trimethinecyanine hydroxide, having the formula:



is prepared as follows:

2,6-dimethyl - 3-(sodiumsulpho-carbomethoxy-methyl)-benzothiazolium bromide (4.2 g.) and 2-( $\beta$ -acetanilidovinyl)-3-ethylthiazolinium bromide (3.5 g.) are dissolved in methanol (35 cm $^3$ ) and the solution is cooled at 0° C. 2.8 cm $^3$  triethylamine are added drop by drop and after one hour stirring under ice-cooling the dyestuff is sucked off and recrystallized three times from a mixture ethanol-water. Absorption maximum: 506 m $\mu$ .

A silver chloride emulsion containing per kg. 15 mg. of this dyestuff is sensitized to 590 m $\mu$  with a broad maximum at 535 m $\mu$ .

## EXAMPLE 13

The dyestuff anhydro-[2-(3-ethylthiazoline)] 2-{3-[p-(omega - sulpho - carbobutoxy) - benzyl] - benzothiazole} trimethinecyanine hydroxide, having the formula:



is prepared as follows:

2-methyl-3-[p-(omega - sodium sulpho - carbobutoxy)-benzyl]-benzothiazolium bromide (5.2 g.) and 2-( $\beta$ -acetanilidovinyl)-3-ethyl thiazolinium bromide (3.5 g.) are dissolved in ethanol (35 cm $^3$ ) and after cooling the solution at 0° C., 2.8 cm $^3$  triethylamine are added. After stirring for one hour under ice-cooling the dyestuff is

45

sucked off and crystallized from ethanol. Absorption maximum: 584 m $\mu$ .

A silver bromo iodide emulsion containing per kg. 15 mg. of this dyestuff is sensitized to 690 m $\mu$  with a broad maximum at 635-640 m $\mu$ .

## EXAMPLE 15

The dyestuff anhydro-[2-(3-ethyl-naphtho-1':2':4:5-thiazole)] - {2 - [3-(omega-sulpho-carbobutoxy)-methylbenzselenazole]} trimethinecyanine hydroxide, having the formula:



is prepared as follows:

2 - methyl - 3 - (omega - sodium sulpho - carbobutoxy-methyl)-benzoselenazolium bromide (5 g.) and 2-( $\beta$ -acetanilidovinyl)-3-ethylnaphtho - 1':2':4:5 - thiazole-para-tolusulphonate (5.5 g.) are dissolved in acetic anhydride (30 cm $^3$ ) and after adding drop by drop 2.8 cm $^3$  triethylamine the solution is brought at boiling temperature for twenty minutes. After cooling, the dyestuff precipitates and is recrystallized from ethanol. Absorption maximum: 584 m $\mu$ .

A silver bromo iodide emulsion containing per kg. 15 mg. of this dyestuff is sensitized to 690 m $\mu$  with a broad maximum at 635-640 m $\mu$ .

## EXAMPLE 16

The dyestuff anhydro{2-[1-ethyl-3-(sulphocarbomethoxy-methyl) - 5,6 - dichlorobenzimidazole]}[2-(3-ethylbenzoxazole)] trimethinecyanine hydroxide, having the formula:



is prepared as follows:

1 - ethyl - 2 - methyl - 3-(sodium sulpho-carbomethoxy-

## 17

methyl)-5,6-dichlorobenzimidazolium bromide (2.4 g.) and 2-(phenylimino - ethylidene) - 3 - ethylbenzoxazoline (1.65 g.) are dissolved in acetic anhydride (20 cm.<sup>3</sup>) and, after the addition of triethylamine (1.4 cm.<sup>3</sup>) left overnight at 20°. The dyestuff is precipitated with ether and recrystallized twice from ethanol and once from diacetone alcohol-water. Absorption maximum: 491 m $\mu$ .

## EXAMPLE 17

The dyestuff anhydro{2 - [3 - sulfo - carbomethoxy-methyl]-4-methylthiazole]}[2 - (3 - ethylbenzoxazoline)]-trimethinecyanine hydroxide, having the formula:



is prepared as follows:

2,4-dimethyl-3-(sodium sulpho-carbomethoxy-methyl)-thiazolium bromide (1.8 g.) and 2-( $\beta$ -acetanilidovinyl)-3-ethylbenzoxazolium iodide (2.2 g.) are dissolved in acetic anhydride (20 cm.<sup>3</sup>), triethylamine (1.4 cm.<sup>3</sup>) is added and the mixture is heated for 2 hours at 80°. After cooling the dyestuff is precipitated with ether and recrystallized three times from ethanol. Absorption maximum: 518 m $\mu$ .

As shown in the above examples, the new methine dyes spectrally sensitizes photographic silver halide emulsions when incorporated therein. Although the new methine dyes are useful especially for extending the spectral sensitivity of the customarily employed gelatino silver chloride, gelatino silver chloro-bromide, gelatino silver bromide, gelatino silver bromo-iodine and gelatino silver chloro-bromo-iodine emulsions, photographic emulsions containing water-permeable colloids other than gelatin, such as agar-agar, zeine, collodion, water-soluble cellulose derivatives, polyvinyl alcohol or other hydrophilic synthetic or natural resins or polymeric compounds, may equally well be sensitized according to the present invention.

To prepare photographic emulsions sensitized according to the invention with one or more of the new methine dyes, the dye, or dyes can be incorporated in the photographic emulsion by one of the methods customarily employed in the art. In practice, it is convenient to add the dyes to the emulsion in the form of a solution in an appropriate solvent. The dyes are advantageously incorporated in the finished, washed emulsions and should be uniformly distributed throughout the emulsion. The concentration of the dyes in the emulsion can vary widely, for example from 1 to 100 mg. per kg. of flowable emulsion and will vary according to the effect desired. The suitable and most economical concentration for any given emulsion will be apparent to those skilled in the art, upon making the ordinary tests and observations customarily used in the art of emulsion making.

The new methine dyes can be incorporated in photographic emulsions the general sensitivity of which has been increased by physical and chemical ripening. An suitable chemical sensitizers may be mentioned the well known sulphur sensitizers such as allylisothiocyanate, allylthiourea, sodium thiosulphate, potassium selenocyanide and the natural sensitizers originating in the gelatin, reducing sensitizers such as the imino-aminomethane-sulphuric acid and the derivatives thereof, and the salts of noble metals such as gold, platinum and palladium.

The photographic emulsions optically sensitized according to the invention may further be supersensitized and/or hypersensitized by one of the methods known to those skilled in the art.

In preparing the photographic emulsions according to the invention, the usual addenda such as antifogging

5

10

15

20

We claim:

1. A methine dye of the formula:



wherein:

Z constitutes the atoms necessary to complete a heterocyclic system selected from the group consisting of benzothiazole, 6-methoxybenzothiazole, 6-methyl benzothiazole, 5-methyl benzothiazole, 5,6-dimethyl benzothiazole, benzoselenazole, benzoxazole, 5-phenyl benzoxazole, 6-methoxybenzoxazole, benzimidazole, 5,6-dichlorobenzimidazole, thiazole and 4-methyl thiazole;

Z' constitutes the atoms necessary to complete a heterocyclic system selected from the group consisting of benzothiazole, benzoselenazole, benzoxazole, benzimidazole, thiazole, naphthothiazole, selenazoline and thiazoline;

d is a positive integer from 1 to 3;

R is a member selected from the group consisting of hydrogen and methyl;

R' is a radical of the formula



wherein A is lower alkylene, and p a positive integer from 1 to 6, and

R'' is a member selected from the group consisting of lower alkyl and



wherein A is lower alkylene, p a positive integer from 1 to 6 and M an alkyl metal atom.

2. Methine dye of formula:



3. Methine dye of the formula:



19

4. Methine dye of the formula:



5. Methine dye of the formula:



20

References Cited in the file of this patent

## UNITED STATES PATENTS

- 5 2,213,995 Riester et al. Sept. 10, 1940  
 2,646,430 Brooker et al. July 21, 1953  
 2,870,014 Brooker et al. Jan. 20, 1959  
 2,892,836 De Stevens June 30, 1959  
 2,892,838 Sprague June 30, 1959  
 2,905,666 De Stevens Sept. 22, 1959  
 10 2,973,264 Nys et al. Feb. 28, 1961

## FOREIGN PATENTS

- 559,840 Belgium Feb. 5, 1958

## OTHER REFERENCES

- 15 Elsevier: "Chemistry of Carbon Compounds," vol. IB, pages 809-10, Elsevier Publishing Co., Amsterdam (1952); QD 251 R 6.